

E. WEINHEIM.

ARTIFICIAL TANNED FABRIC WITH FINISH COATING AND PROCESS OF MAKING SAME.

APPLICATION FILED OCT. 3, 1908.

926,525.

Patented June 29, 1909.



Witnesses:

Alfred Schenck  
George Lilschen

Inventor  
Emil Weinheim  
By His Attorney  
Leonard Day.

EMIL WEINHEIM, OF NEW YORK, N. Y.

## ARTIFICIAL TANNED FABRIC WITH FINISH COATING AND PROCESS OF MAKING SAME.

No. 926,525.

Specification of Letters Patent.

Patented June 29, 1909.

Application filed October 3, 1908. Serial No. 455,951.

*To all whom it may concern:*

Be it known that I, EMIL WEINHEIM, a citizen of the United States, and a resident of the borough of Manhattan, county, city, and State of New York, have invented certain new and useful Improvements in Artificial Tanned Fabrics with Finish-Coating and Processes of Making Same, as set forth in the following specification.

10 This invention relates to an artificial fabric with a finish coating and to the process of making same.

It relates more particularly to a suitably colored finish coating and the process of forming the same on a particular kind of artificial leather which in itself is specifically claimed as well as the process for making it in applicant's copending application, Serial No. 455,953, filed October 3, 1908 for artificial tanned fabric and process of making the same.

An object of the invention is to insure the firm adherence of a suitable patina or colored coating to a foundation fabric particularly 25 the artificial tanned fabric referred to.

A further object is to provide such a coating, which is water-proof not only on its finished surface but which is water-proof interiorly where it adheres to and contacts 30 with the fibers of the body fabric.

The invention applies both to the process of applying such a coating, to the ingredients in combination in the coating, and to the fabric so coated as an article of manufacture.

35 An object of the invention is to provide for the application of a suitable patina, which is more or less soluble before application, to the body fabric but which is rendered insoluble after its application to such body 40 fabric.

More in general an object of the invention is to improve surface finished fabrics to be used as substitutes for tanned and finished leather in the arts; to provide such a product 45 that the finish coating will not peel off under the action of moisture; to provide such a finished fabric which will have the structural qualities, as durability, suppleness and toughness of tanned animal leather and will 50 also have the surface appearance of the outside surface of finished tanned leather.

To the above end the use of free dichromate of potassium in and about the fibers of a suitable body fabric is employed preparatory 55 to applying any suitable patina which may it-

self be soluble but which will be rendered insoluble by the dichromate of potassium. It is to be understood also, that the use of a patina such as described herein not necessarily upon a fabric impregnated with dichromate of potassium is useful and will produce a useful product.

The above and further objects of this invention will be set forth in the accompanying claims and will be apparent from the following description which may be read in connection with the accompanying drawing which forms part of this application and in which the single figure is an enlarged, exaggerated cross section through the finished product.

In practicing this process it is desirable to provide first a mat or batting of fibrous substance, preferably cotton fiber. It has been found that long fibers increase the strength 75 of the finished product. It has also been found that a substantially equal mixture of long and short fibers results in a finished product comparing in strength, durability, etc., very favorably with one made up from 80 a body of entirely long fibers. It is of course, to be understood that the longer fibers are more expensive than the shorter. This feature of mixing long with short fibers has the commercial advantage of cheapness 85 without sacrificing strength and durability. Preferably, therefore, various proportions, according to the desired strength of the ultimate product, of long and short cotton fibers are matted into a batting of uniform 90 thickness which may vary according to the desired thickness of the finished product, so that its weight per square yard may vary satisfactorily from 125 grams to 800 grams 95 or more or less as desired. The batting may be formed into suitable strips or rolled strips as convenient. The next step is to provide 100 an aqueous solution of dichromate of potassium, say a three to a ten per cent. solution according to the amount of deposit required, and as will hereinafter be apparent. This dichromate of potassium solution is sprinkled uniformly upon the batting described so as not to destroy its character as a strip of batting. During this process a suitable supporting surface for the batting is desirable. 105 The batting then should be dried after a complete impregnation of all its fibers has been accomplished by the sprinkling. Care should be taken that the batting resume its 110

original fluffiness or looseness of texture subsequent to drying after being impregnated with the solution of dichromate. Care should also be taken that the impregnation with dichromate is uniform and complete insuring a uniform crystalline deposit of dichromate upon each and all of the fibers of the matting after suitable drying has taken place. The batting so impregnated with dichromate of potassium and rendered dry and fluffy, is termed a batting or body of dichromatized vegetable fibers. For the next step the batting may be cut into sheets or strips of suitable size, it being borne in mind that the size and shape of a finished sheet of fabric will resemble that of the initial sheet of batting. Metallic plates of a size slightly larger than the sheets of batting, thus provided, are furnished. These metallic plates may be of zinc or other suitable metal, and it may be desirable that they be sufficiently thin to provide a certain degree of flexibility. An improved leatherfying composition for saturating the sheets of batting is then compounded, as follows, or the same should have been previously prepared and ready at hand at this step of the process.

The following ingredients are mixed and combined in suitable proportions easily determined by experiment and subject to considerable variation but such that the resulting mass is sufficiently fluid for coating purposes when at a temperature of from sixty to eighty degrees Fahrenheit. The parts are as follows: 1. Viscous animal parts, such as bone glue, gluten and other glutinous matter of animal origin. 2. Vegetable oils, such as palm oil, olive oil and others. 3. Hydrocarbons, such as paraffin, vaseline, bitumen or others. 4. Animal fats, such as tallow, suet and others. 5. Metallic salts, such as hydrated oxid of zinc, potassium, lead and aluminum. 6. Suitable saponifying agents, such as sodium and potassium alkalies.

It is well to keep the viscous animal parts in water previously to use, so as to aid their ready fusibility and manipulation. A suitable vessel with means for heating the same is provided and may be a steam heated caldron. The first five sets of ingredients, it being understood that one or more of the specified ingredients in each set can be used, are kneaded and mixed together under the influence of heat, until a uniform mixture is accomplished. The saponifying agent should then be added and heating continued until satisfactory saponification of the mixture has been accomplished. The preferable temperature during saponification is from eighty to ninety degrees Fahrenheit.

With the composition above described or with any composition having suitable qualities maintained at an even temperature of from sixty to eighty degrees Fahrenheit, the same is suitably applied to the metallic

plates which have been previously described. The coating should be uniform on both surfaces of the plates and its thickness will correspond somewhat to the viscosity of the coating composition.

70

A tier of alternating coated plates and sheets of batting may be built up to a suitable total thickness convenient for manipulation. The bottom of the tier may be a metal plate coated only on its top surface and the top of the tier a metal plate coated only on its bottom surface. The tier may be placed in a suitable press maintaining the plates and sheets horizontal between parallel pressure applying devices. The tier is then subjected to a gradual pressure under the influence of heat. It is desired that the entire tier be heated to approximately 70° Fahrenheit throughout or even more. The heat and pressure is continued until the dichromate of potassium has insolubilized or effected the insolubility of the saturating leatherfying composition and until said composition has saturated the entire thickness of each sheet of batting. Dichromate of potassium is employed as a suitable insolubilizing agent, although it is to be understood that any agent having a similar effect may be employed. At this stage in the process the body of batting will have been compressed to a much less thickness than it was initially. The tier of plates and sheets should then be removed from the heated press and be subjected to pressure in a cooling atmosphere. Then they are taken out; the sheets are separated from the metal plates and dried, each sheet being exposed individually to the influence of a drying atmosphere. It is found that this subsequent drying is useful to expel moisture which is no longer combined in the saturating leatherfying composition, but appears to be in a free state. After being suitably dried the resultant sheets form a body fabric to be provided with a finish coating of patina of any desired color.

If the amount of dichromate of potassium, with which the batting heretofore was impregnated, was merely sufficient to provide for the water-proofing of the saturating leatherfying composition, it will be desirable to incorporate or intimately relate free dichromate of potassium with the surface fibers of the surface of the body fabric to be provided with the finish coating. This may be accomplished in any suitable manner as by sprinkling with a solution of dichromate of potassium and drying out the water to cause a deposit of the dichromate in and about the surface fibers of the fabric. It may, however, be desirable to increase the percentage of the dichromate of potassium used in the fiber batting above that necessary to waterproof the saturating leatherfying composition referred to. This may be accomplished by

75

80

85

90

95

100

105

110

115

120

125

130

135

increasing the strength of the solution of dichromate of potassium sprinkled on to and into the batting or may preferably be accomplished by sprinkling the batting a second time after it has once been well saturated with the solution of dichromate of potassium and once dried out, and then drying it a second time. This second sprinkling will increase the proportion of deposited dichromate of potassium relatively to the fiber batting particularly about the surface fibers of the surface of the batting. The complete sheet or body fabric made up from a batting so treated with dichromate of potassium will 10 contain a sufficient amount of free dichromate of potassium about its surface fibers satisfactorily to water proof the finish coating of patina which will presently be described.

20 *Illustrative ingredients for finish coating or patina.*—The following ingredients are mixed and combined in suitable proportion easily determined by experiment and subject to considerable variation but such that the resulting composition is sufficiently fluid for coating purposes when at a temperature say from 60° to 80° Fahrenheit. The parts are as follows: 1. Suitable coloring matters, preferably mineral. 2. Viscous animal parts, such as bone glue, gluten and other glutinous matter of animal origin. 3. Vegetable oils, such as palm oil, olive oil and others. 4. Hydro-carbons, such as paraffin, vaseline, bitumen or others. 5. Animal fats, such as tallow, suet and others. 6. Metallic salts, such as hydrated oxid of zinc, potassium, lead and aluminum. 7. Suitable saponifying agents, such as sodium and potassium alkalies.

40 The above is merely an illustrative composition for a suitable patina and it is to be understood that certain ingredients may be substituted by equivalents or omitted according to the product desired. The patina may be formed conveniently in a suitable vessel suitably heated.

50 The surface of the body fabric to be finished is painted over one or more times in accordance with the homogeneousness of the coloring desired. The painting may be accomplished by the aid of suitable brushes which travel backward and forward in the direction of movement of the sheet to be coated which may be caused to travel by means of suitable rollers. During the painting process the sheet should be maintained suitably heated to aid in rendering the coating insoluble by means of the dichromate of potassium. It is desirable that the patina be thoroughly rubbed into the surface of the sheet so that it adheres to and embeds itself about and over the surface fibers. In the drawing 1 indicates the body fabric, while 2 indicates the patina shown in intimate relation with the surface fibers of the body fabric 1 along the surface 3 of the body fabric 1. It should be noted that the composition of the patina for the finish coating is substantially the same as that of the leatherfying composition for saturating the sheets of batting except for the admixture of suitable coloring materials. The coating of patina therefore not only adheres and embeds itself about the surface fibers of the body fabric but incorporates itself with and forms a dense surface coating for the body of and of substantially the same character as the body fabric itself. A considerable degree of pressure is applied to the patina coated surface of the body fabric when the coating is 70 painted on. After the desired homogeneousness of color for the coating has been obtained the coated sheet may be brought into the drying room as before and be maintained at a moderate temperature, say from 70° to 85° Fahrenheit, where it is thoroughly dried. After thus being dried the colored side of the sheet may be varnished in accordance with the degree of luster desired with a varnish composed of a mixture of casein substance, 80 vegetable oils, a fatty acid such as olein and the entire mixture saponified by suitable alkali. This coat of varnish is indicated by 4. The sheet should then be dried again, after which it may be calendered between metallic plates such as smooth zinc plates covered with homogeneous felt over which is rolled a cylinder of such a weight as to apply the degree of pressure desired for calendering. The cylinder may first be rolled over 90 the felt and then over the metal plate with the coated surface of the sheet beneath the plate. The sheet so calendered may thereafter be embossed with any suitable design even in very high relief. The embossing 100 may be accomplished by any suitable process as by the use of a stereotype or galvanoplastie plate provided with the desired design and by means of the calendering cylinder heretofore mentioned or by means of a suitable heated press. The product after calendering is satisfactory for use as a substitute for finished tanned leather in the arts and is satisfactorily water-proof throughout. It 110 has been found that a denser surface may be 115 formed over the surface of the patina by applying a solution of formaldehyde and alcohol. After this is done the product should again be dried to expel the water and alcohol. 120 It is to be understood that the patina described may be applied to the artificial tanned leather fabric without providing the surplus deposit of dichromate of potassium on the surface of the fabric to be coated and then relying merely upon the similarity of 125 the composition of the patina to that of the saturating composition in the body fabric to insure satisfactory adherence for the colored finish coat, or patina. In this case it is 130 more desirable to apply the final coat of

formaldehyde described above although that may be omitted.

Although this invention is set forth in detail, it is understood that the various steps 5 may be varied without departing from the invention.

What is claimed and what is desired to be secured by United States Letters Patent, is:

1. The process of making artificial tanned 10 fabric with a finish coating comprising, the production of a soft fluffy batting of vegetable fibers impregnated throughout with dichromate of potassium; forcing a more or less soluble leatherfying composition into 15 said batting under continued pressure and heat to effect the insolubility of said leatherfying composition in and about the fibers of the batting; drying the so saturated batting; coating a surface of the dried fabric with a 20 patina comprising said leatherfying composition suitably colored; intimately relating said patina about the surface fibers of said 25 fabric; and compacting the said coating of patina and rendering it insoluble by means of heat and surface pressure.

2. The process of making artificial tanned 30 fabric with a finish coating comprising, producing a body fabric composed of vegetable fibers and a saturation of a leatherfying composition rendered insoluble; incorporating dichromate of potassium in solution in and about the surface fibers on the surface to be coated; drying out the water from said dichromate solution to precipitate dichromate 35 of potassium in and about the said surface fibers; applying a patina of similar composition to said leatherfying composition as a coating to said surface; and compacting the same and effecting the insolubility of the 40 same by heat and pressure.

3. The process of making artificial tanned 45 fabric with a finish coating comprising, producing a body fabric of vegetable fibers saturated with a leatherfying composition ren-

dered insoluble by an excess of dichromate of potassium so that free dichromate of potassium will remain distributed about the fibers of said fabric; drying out the moisture from the so saturated fabric; and brushing on a surface coating under heat and pressure 50 of a patina of similar composition to that of the leatherfying saturating composition.

4. As an article of manufacture, the product of the process described, a sheet of artificial tanned leather having a finish coating 55 and comprising a body of matted and dichromatized vegetable fibers; a body filling of leathery composition as described insolubilized *in situ* in and about the said fibers and forming a close union with the said fibers 60 throughout the said body; and a dense surface coating of colored patina having a similar composition to that of the said leathery composition and directly incorporated therewith and with the surface fibers of the said 65 fabric.

5. As an article of manufacture, the product of the process described, a sheet of artificial tanned leather having a finish coating and comprising a body of matted and dichromatized vegetable fibers; a body filling of leathery composition of viscous and leathery animal parts, oils, animal fats, metallic salts and an alkali, as described, insolubilized 70 *in situ* in and about the said fibers and forming a close union with the said fibers throughout the said body; and a dense surface coating of patina having a similar composition to that of the said leathery composition and directly incorporated therewith and with the surface 75 fibers of the said fabric.

In testimony whereof, I have signed my name to this specification in the presence of two subscribing witnesses.

EMIL WEINHEIM.

Witnesses:

LEONARD DAY,  
EDSON B. SAMMIS.